

# UNITED STATES PATENT OFFICE.

HARRY WILLIAMS CHARLTON, OF OTTAWA, ONTARIO, CANADA.

## MATCH-IGNITION COMPOSITION.

1,089,902.

Specification of Letters Patent. Patented Mar. 10, 1914.

No Drawing.

Application filed May 13, 1911. Serial No. 627,066.

*To all whom it may concern:*

Be it known that I, HARRY WILLIAMS CHARLTON, a citizen of Canada, residing at Ottawa, in the county of Carleton and Province of Ontario, Canada, have invented new and useful Improvements in Match-Ignition Composition, of which the following is a specification.

This invention pertains to non-poisonous substitutes for yellow phosphorus, and relates exclusively to salts of this element in whose molecules are one or more atoms of nitrogen. As a class these salts are stable, but, owing probably to the slight affinity of nitrogen for other elements, they are readily acted on by powerful oxidizing agents. They yield match ignition compositions which strike on any surface, or by varying the proportions of the ingredients in the mixture, excellent safety matches may be produced.

Considered as a class the salts of phosphorus containing nitrogen are stable voluminous solids that are easily prepared and can be handled without the slightest inconvenience. Most of these possess to a greater or less degree the ability to enter into chemical action with potassium chlorate, (when present in formed match heads), upon the application of slight friction. On its quality in this respect depends the value of any easily oxidizable material in match ignition compositions. This is not a characteristic common to easily oxidizable materials as a class, and seems to be entirely absent in many materials that are ordinarily oxidized with the greatest ease.

When incorporated with the ordinary constituents of match ignition compositions, such as chlorate of potash, ground glass, a filler and solution of glue, and the whole allowed to set, it is observed that the nitrogenous compounds of phosphorus act as efficient oxidizable materials. At the same time the addition of other easily oxidizable

materials has a very beneficial effect. If a small amount of sesquisulfid of phosphorus or amorphous phosphorus be present the sensitiveness is materially increased.

The following is given purely as an example of a formula that might be used.

|                               |   |        |
|-------------------------------|---|--------|
| Phosphorus nitrogen compound  | 4 | parts. |
| Potassium chlorate            | 3 | "      |
| Powdered glass                | 1 | part.  |
| Iron oxid                     | 1 | "      |
| Zinc oxid                     | 1 | "      |
| Glue (60% solution in water.) | 4 | parts. |

Phospham has been particularly referred to but it simply stands as a representative of a large class of compounds that are equally efficient. Among the easily oxidizable materials that may be associated with it are sulfids of phosphorus, amorphous and also the more recently discovered scarlet phosphorus. The first two may easily be present as impurities.

I claim:

1. In a match ignition composition a nitrogenous phosphorus compound, an oxidizing agent and chemically inert material.

2. In a match ignition composition a nitrogenous phosphorus compound, an oxidizing agent, a filler, frictional matter and a binding agent.

3. In a match ignition composition a nitrogenous phosphorus compound containing as impurities other easily oxidizable materials, potassium chlorate, oxid of zinc, powdered glass and glue.

4. In a match ignition composition phospham containing stable sulfids of phosphorus as impurities, an oxidizing agent, a filler, frictional matter and a binding agent.

Ottawa, May 10th, 1911.

HARRY WILLIAMS CHARLTON.

Witnesses:

H. O. FALKINS,  
A. IRWIN.